

Patented Apr. 5, 1927.

1,623,048

# UNITED STATES PATENT OFFICE.

JUSTIN D. CROSBY, OF PAWTUCKET, RHODE ISLAND, ASSIGNOR TO J. D. CROSBY CO.,  
OF PAWTUCKET, RHODE ISLAND, A CORPORATION OF NEW YORK.

## PROCESS OF FINISHING COLD-ROLLED STEEL.

No Drawing.

Application filed May 4, 1922. Serial No. 558,532.

This invention relates to a process of finishing cold-rolled strip steel or flattened wire, and has for its main object and feature the production of steel of a very high and unusual lustre combined with the requisite degree of hardness or temper.

Low carbon cold-rolled strip steel is used extensively in the art for making flat, bent, drawn or spun metal products and is generally produced from hot-rolled strips. While cold-rolling, as heretofore practiced, produces a certain amount of smoothness and brightness of the steel there are certain exacting uses to which the steel is sometimes put that require a smoothness and brightness that has heretofore been obtained only by subjecting the steel, after cold-rolling, to a polishing operation and steel that has been so treated is sometimes called "polished steel."

I have found a method whereby the polishing operation may be dispensed with and steel of unusual lustre may be obtained during the process of cold-rolling. The temperature, that is the hardness or softness of the steel and the amount of reduction in thickness are, however, bound up with the process of rolling the steel, repeated rollings increasing the hardness of the material and reducing its thickness, and therefore the problems of hardness, the reduction, and lustre are intermingled and must be coordinated.

I find that, by cleaning and drying the steel so as to render its surface as free from foreign matter as possible, the steel may have an unusual lustre imparted to it by subjecting it to a cold-rolling operation by means of dry rolls of hardened steel.

By "dry rolls" is meant that contrary to the usual practice no lubricant is employed on the surface of the rolls. The result of this rolling is that the rolls act against the steel "metal to metal" with no intervening film of lubricant or other matter and the fine surface-texture of the rolls is therefore imprinted upon the steel giving it a high and unusual lustre. The rolling of course also reduces the thickness of the material and increases its hardness.

The cleaning and drying of the steel may be produced in various ways as by heat, chemicals, mechanical scrubbing or otherwise, one method consisting in combining the step of cleaning and annealing or

softening. These different operations must, however, be properly coordinated with the dry rolling and the steps will be varied as to their order with respect to the dry rolling and as to their character to obtain different degrees of hardness with the same character of lustre.

I have found that a certain degree of hardness which we call in our shop TH and TQ (three and a half and three and three quarters) may be obtained combined with the requisite lustre by proceeding in the following manner.

The hot-rolled strip steel is reduced to a proper thickness and is then cleaned by being pickled and limed and is then given a number of passes in the usual manner, the rolls being supplied with a lubricant. This produces a well known form of strip steel with a smooth, bright surface. The next steps in the process consist in annealing and keeping clean and bright the strip so formed. If any foreign matter gets on this strip it should be cleaned off. Assuming that this strip is clean and bright, it is then passed between the hard steel, highly polished rollers, without any lubricant or other foreign matter, so that there is a clean, direct metal to metal contact between the strip and roller with what is known as a "light pass" rolling which reduces its thickness about one one thousandth of an inch and imparts a polish with a high lustre or "satin finish" which requires no subsequent polishing. I have found that the best results are obtained with two such light passes with strips about two one hundredths of an inch in thickness.

Having thus described my invention, what I claim is:

The method of imparting a high lustre or polish to steel strips which consists in reducing the steel to the requisite thickness and giving it a preparatory treatment of cleaning, drying and cold rolling with oiled rollers and thereafter annealing and then passing this clean and annealed strip with a light pass between dry, highly polished steel rollers which slightly reduce its thickness and impart a high lustre or polish.

Signed at Pawtucket, in the county of Providence and State of Rhode Island, this 10th day of April, 1922.

JUSTIN D. CROSBY.